

## UNITED STATES PATENT OFFICE

BERKELEY L. HATHORNE, OF NEW YORK, N. Y., ASSIGNOR TO TUBIZE CHATILLON CORPORATION, A CORPORATION OF DELAWARE

## PROCESS OF DYEING RAYON

No Drawing.

Application filed June 3, 1929. Serial No. 388,187.

This invention relates to a process of dyeing rayon in filament or fabric form with oil-soluble dyes and colors, and more particularly to the dyeing of delusterized rayon 5 filaments or fabrics.

In the various processes of preparing rayon it has been found that there is incorporated throughout the filaments formed an oil, fat or wax, and this is especially true 10 in many delustered rayon fibers.

This process is of particular value to the dyeing of delustered rayon by means of the so-called oil-soluble dyes or colors, and it is proposed to dye the globules of oils, fats 15 or waxes in the rayon and leave the rayon fiber either undyed or only moderately stained. A few of the so-called oil-soluble colors will dye ordinary rayons and other cellulose fibers, and the present invention 20 includes these colors.

Due to inherent manufacturing difficulties encountered in the preparation of rayon filaments, there is considerable difference 25 from skein to skein, and while it is not at present known whether these differences in the filaments are physical or chemical, the resultant fabrics woven from these filaments are quite difficult to dye with any degree of uniformity or level. Such rayon fabrics at 30 present, after dyeing, exhibit dark and light strands, which, of course, detracts from their appearance.

Fundamentally, the present process contemplates the placing of the so-called oil-soluble dyes or colors in an aqueous solution 35 in such a manner that the dyes or colors will uniformly stain the rayon to the correct depth or level, and in carrying out the process the minute globules or oils, fats or waxes 40 in the rayon are dyed, while the cellulose fiber is either left entirely undyed or only moderately stained.

In carrying out the process, a novel boiling bath is utilized in which the oil-soluble 45 dyes are intimately associated.

The following is a specific example of a dye bath which has been most successfully used in dyeing delustered rayon:

2 grams of benzol or other organic solvent 50 are added to 10 grams of sulfonated castor

oil or other soap stock.  $\frac{1}{2}$  gram of any suitable oil-soluble dye or color is then added to the above and thoroughly mixed. A boiling solution consisting of 5 grams of soap and 25 grams of water, or in all 30 55 grams of solution, is added to the color solution and thoroughly agitated, after which 2 liters of water containing 5 grams of soap kept at a boiling temperature are added to the initial boiling solution. By the term 60 rayon I intend to include acetate cellulose.

The boiling bath so formed is placed in a suitable vat in which is immersed 100 grams of rayon filaments or fabrics. The rayon is treated for a period of approximately thirty minutes, during which time the bath is maintained at a temperature of approximately 200° F., after which it is removed from the bath and washed and dried in the well-known manner. Preferably, 65 though not necessarily, the combined boiling and dyeing bath is agitated or stirred during the period of treatment.

Thus it will be seen that a stable boiling and dyeing bath is produced in which the 75 oil-soluble color is intimately dissolved and one in which normal dyestuffs which are not oil-soluble may be advantageously used. Furthermore, it is possible with this process to dye delusterized rayon and another cellulose fiber simultaneously in the same bath, using the oil-soluble colors, or a combination of oil-soluble colors and ordinary dyestuffs, so that the different fibers are cross dyed or two-toned effects are produced. 80 85

Rayon filaments or fabrics dyed in accordance with this process have a uniform depth or level of color as there is a perfect combining of the dyestuffs with the minute globules of oils, fats or waxes, which are 90 uniformly distributed throughout the fiber, while the fiber itself remains undyed or only moderately stained.

What is claimed is:

1. As a new article of manufacture, a 95 rayon filament in which only the oils, fats and waxes contained therein have been dyed with oil-soluble colors.

2. The process of dyeing the oily constituents of delustered rayon which consists in 100

immersing said rayon in a boiling bath containing oil-soluble colors.

3. The process of dyeing the oil constituents of delustered rayon which consists in immersing said rayon for a period of approximately thirty minutes in a boiling bath containing oil-soluble colors.

4. The process of dyeing the oily constituents of delustered rayon which consists in immersing said rayon in a boiling bath containing oil-soluble colors, said bath being maintained at a temperature of approximately 200° F.

5. The process of preparing a rayon dye bath for dyeing the oily constituents of rayon which consists in dissolving an oil-soluble color in an organic solvent and soap mixture, adding an aqueous soap solution thereto, agitating the two mixtures together and subsequently adding a second heated dilute soap solution thereto and agitating the combined mixtures.

6. The process of imparting color to rayon which consists in dyeing only the oils, fats and waxes contained therein.

25 In testimony whereof I affix my signature.

BERKELEY L. HATHORNE.

#### CERTIFICATE OF CORRECTION.

Patent No. 1,913,987.

June 13, 1933.

BERKELEY L. HATHORNE.

It is hereby certified that error appears in the printed specification of the above numbered patent requiring correction as follows: Page 1, line 39, for "or" first occurrence read "of"; and lines 60 and 61, strike out the words "By the term rayon I intend to include acetate cellulose." and insert the same after "stained." in line 93; and that the said Letters Patent should be read with these corrections therein that the same may conform to the record of the case in the Patent Office.

Signed and sealed this 15th day of August, A. D. 1933.

Acting Commissioner of Patents.

(Seal)

immersing said rayon in a boiling bath containing oil-soluble colors.

3. The process of dyeing the oil constituents of delustered rayon which consists in immersing said rayon for a period of approximately thirty minutes in a boiling bath containing oil-soluble colors.

4. The process of dyeing the oily constituents of delustered rayon which consists in immersing said rayon in a boiling bath containing oil-soluble colors, said bath being maintained at a temperature of approximately 200° F.

5. The process of preparing a rayon dye bath for dyeing the oily constituents of rayon which consists in dissolving an oil-soluble color in an organic solvent and soap mixture, adding an aqueous soap solution thereto, agitating the two mixtures together and subsequently adding a second heated dilute soap solution thereto and agitating the combined mixtures.

6. The process of imparting color to rayon which consists in dyeing only the oils, fats and waxes contained therein.

25 In testimony whereof I affix my signature.

BERKELEY L. HATHORNE.

#### CERTIFICATE OF CORRECTION.

Patent No. 1,913,987.

June 13, 1933.

BERKELEY L. HATHORNE.

It is hereby certified that error appears in the printed specification of the above numbered patent requiring correction as follows: Page 1, line 39, for "or" first occurrence read "of"; and lines 60 and 61, strike out the words "By the term rayon I intend to include acetate cellulose." and insert the same after "stained." in line 93; and that the said Letters Patent should be read with these corrections therein that the same may conform to the record of the case in the Patent Office.

Signed and sealed this 15th day of August, A. D. 1933.

Acting Commissioner of Patents.

(Seal)

**CERTIFICATE OF CORRECTION.**

**Patent No. 1,913,987.**

**June 13, 1933.**

**BERKELEY L. HATHORNE.**

It is hereby certified that error appears in the printed specification of the above numbered patent requiring correction as follows: Page 1, line 39, for "or" first occurrence read "of"; and lines 60 and 61, strike out the words "By the term rayon I intend to include acetate cellulose." and insert the same after "stained." in line 93; and that the said Letters Patent should be read with these corrections therein that the same may conform to the record of the case in the Patent Office.

Signed and sealed this 15th day of August, A. D. 1933.

**(Seal)**

**Acting Commissioner of Patents.**